

## UNITED STATES PATENT OFFICE

2,033,974

## FERRO-CARBON-TITANIUM ALLOY

George F. Comstock, Niagara Falls, N. Y., assignor  
to The Titanium Alloy Manufacturing Company, New York, N. Y., a corporation of Maine

No Drawing. Application June 20, 1935,  
Serial No. 27,543

8 Claims. (Cl. 75—1)

This application is a continuation in part of my copending application for patent filed March 27, 1934 Serial No. 717,574.

5 My invention relates to a new and improved type of ferro-carbon-titanium alloy for use in treating molten steel for the purpose of fluxing and assisting the removal of gaseous and other objectionable impurities.

10 Titanium alloys previously available commercially are of two general classes—(1) high-carbon alloys containing 6 to 9% carbon; and (2) low-carbon alloys containing effective amounts of aluminum or silicon in addition to the titanium.

15 For treating very low-carbon steel or pure iron, such as is used for sheets that must be very ductile, the ordinary low-carbon ferrotitanium alloys are not used to advantage, either on account of their high cost, or because of their high silicon or aluminum contents.

20 The reason for the objection to a high silicon content is that such steels or ingot-irons are best cast in the form of effervescing ingots, in which the evolution of gas on solidification causes the outer skin to solidify in an especially clean and pure state so that the highest ductility is attained; the presence of silicon in appreciable amounts in the steel interferes too much with the proper effervescence and structure of the ingots.

25 The reasons for the unsuitability of the other kind of low-carbon ferrotitanium alloy (of low silicon content), which has heretofore been available commercially for use in low-carbon steels, are chiefly that its cost is too high owing to the necessity for using considerable aluminum in its 30 manufacture, and also in part because of the unavoidable presence in the alloy of an effective amount of aluminum which has the same undesirable action on effervescing steel as that of silicon which I just described.

35 For effervescing low-carbon steel, it has generally been found advantageous to use the high-carbon ferrotitanium, or ferro-carbon-titanium as it is known commercially, which can be made much cheaper than the aluminum-reduced low-carbon alloy. It is added in rather small amounts to the molten steel a short time before pouring, and acts as a mild deoxidizer and scavenger to 40 control the effervescence of gas on solidification of the steel and to produce ingots of the best possible form, structure, and cleanliness.

45 This commercial ferro-carbon-titanium, although sufficiently free from silicon and aluminum to be satisfactory as an addition to effervescing steel, has suffered, up to the time of my present invention, from the disadvantage of too high a carbon content for use in the making of the present-day extremely low carbon steels.

50 The steels of this low-carbon type which are now made for rolling into sheets that must be formed cold into intricate shapes, such as auto-

mobile bodies, must have the lowest possible carbon content in order to permit the necessary distortion without cracking. After the addition of commercial high-carbon ferro-carbon-titanium to this steel, it is often found that the carbon content of the resulting steel is appreciably increased on account of the additional carbon added in the titanium alloy; hence an undesirable limit is imposed on the amount of titanium added so as not to get too much carbon in the steel. 5

10 The common high-carbon ferro-carbon-titanium alloy heretofore in commercial use contains about 15 to 18% titanium, 6 to 9% carbon, 2 to 3% silicon, and 1 to 2% aluminum.

15 In spite of statements published in the early years of the titanium alloy industry to the effect that alloys of this nature contained free titanium and free carbon, it is now definitely established that the affinity of titanium for carbon is so very strong that practically all the titanium in such 20 an alloy combines with carbon, to form the carbide (TiC), which contains 48 parts by weight of titanium to 12 parts by weight of carbon. High-carbon ferro-carbon-titanium, therefore, consists structurally of titanium carbide in a matrix similar 25 to gray cast iron, and also contains from 2 to 4% excess carbon, since the carbon content of the alloy is well over one-fourth of the titanium content. This excess carbon, as shown by chemical analysis and by the dark fracture of the alloy, 30 occurs largely in the form of graphite.

35 Several methods have been tried in the past to produce alloys similar to commercial ferro-carbon-titanium except with a lower carbon content, but the products of such methods invariably suffered from serious objections which rendered them unsuitable for use as sources of titanium for the treatment of low-carbon effervescing steel. Methods involving the use of silicon or aluminum either to replace carbon as a reducing agent for 40 the titanium ore, or to drive out the carbon from the molten alloy by precipitation, gave products too high in those elements, and hence are unsatisfactory as hereinbefore explained.

45 The method of boiling out the carbon from the molten bath of alloy, after its reduction from the ore, by ore additions as commonly practiced in the refining of steel, has not been commercially successful, since when the carbon is really lowered in this way, the titanium is at the same 50 time removed from the alloy either by oxidation or by precipitation of an infusible nitride in the furnace, so that the fluid low-carbon alloy thereby produced is of such a low titanium content as to be commercially worthless.

55 By the improved method which is hereinafter described for the production of the alloy constituting the subject of my invention, I have succeeded in making regularly on a large scale and at a low cost a ferro-carbon-titanium with 60

the desired titanium content between 17 and 23%, with carbon from 1.5 to 5%, and with not over 3% of silicon, aluminum, or other undesirable impurities. The carbon content is held below one-fourth of the titanium content so as to ensure the practical absence of graphite from the alloy, and this product has been found after industrial tests entirely suitable as a source of titanium for the treatment of effervescent steels, similar to ingot iron, of the very lowest carbon content.

My improved lower-carbon ferro-carbon-titanium alloy is preferably made in a single-phase carbon-lined electric furnace, similar to the furnace used for the regular high-carbon alloy, except that it is operated so that carbon is not absorbed from the furnace lining. The charge is composed of 350 pounds ilmenite, 250 pounds steel scrap, and 185 pounds anthracite coal. Current is supplied through a single electrode, at a potential of 50 volts, and regulated to use about 15,000 amperes. The absorption of carbon from the furnace is prevented by omitting a portion or all of the steep scrap from the first few charges so that the excess of ilmenite produces a furnace lining of a refractory titanium compound. By careful maintenance of this high-titanium lining, the furnace may be used for a very much larger number of heats without renewal of the crucible, than has heretofore been possible ordinarily in making the high-carbon alloy.

About half an hour before tapping a finished charge, an addition of 20 to 40 pounds of fine ilmenite ore may be advantageously made to the molten bath so as to produce a boil which assists in lowering the carbon content. This addition may be omitted, however, if the furnace is producing an alloy of sufficiently low carbon content without it, or if necessary the addition of ilmenite may be increased to as much as 100 pounds.

The finished product of this process is a homogeneous melt, and may be cast readily from the furnace. Such alloy solidifies in the form of a dense, solid, crystalline mass, free from the porosity that characterizes the common high-carbon ferro-carbon-titanium alloys. My new alloy is sufficiently hard and lacking in toughness to be crushed fairly readily to the size demanded for additions to molten steel, and when so crushed it exhibits on its surfaces a bright or light-gray fracture free from any black coloration such as is produced by the graphite in the high-carbon alloy. In my alloy the carbon content is substantially all in the combined form with any graphite below 0.2%.

An analysis of an average sample from a large number of casts of my improved lower-carbon ferro-carbon-titanium gave results as follows:

|            | Per cent |
|------------|----------|
| Titanium   | 19.75    |
| Carbon     | 4.45     |
| Silicon    | 2.56     |
| Aluminum   | 1.30     |
| Manganese  | 0.08     |
| Chromium   | 0.073    |
| Phosphorus | 0.023    |

The balance of my new alloy is substantially iron, with unimportant traces of copper, nickel, zirconium, sulphur, nitrogen, etc. All components other than iron, carbon, and titanium are derived from impurities in the ore, scrap, or coal of the charge used in the furnace, and are not

intentionally introduced, but must be controlled within reasonable limits.

By decreasing the proportions of iron and carbon in the charge, an alloy of still lower carbon content may be made, while preserving in other respects the characteristics of the alloy herein described. For example, alloys containing about 24% titanium and 1.84% carbon have been produced in the course of my experiments connected with the development of this new alloy. If the carbon is reduced too low, however, difficulties are encountered either from nitride formation, making the alloy too viscous and difficult to tap from the furnace, or from solution of the high-titanium furnace-lining which results in preventing the production of low-carbon alloy in subsequent operations. For these reasons it has not been found practical as yet to produce regularly alloys with the proper titanium content of from 15 to 25% and less than about 2% carbon by this method.

A satisfactory product which fulfills the requirements for use in very low carbon steel as herein described, and so is included within the limits of my invention, contains 15 to 25% titanium, 1.5 to 5% carbon, less than 3.5% silicon, less than 3% aluminum, and with the balance substantially iron. My preferred composition is 18 to 22% titanium, 3 to 4.5% carbon, 1 to 3% silicon and 0.5 to 1.5% aluminum, with the balance substantially iron, it being impractical to use sufficiently pure ore and coal to secure silicon and aluminum contents below these limits which I have given. They are low enough however to permit the alloy to be used in effervescent or rimming steel without interfering with the proper evolution of gas in the molds.

The carbon content of my new ferro-carbon-titanium alloy should be practically all in the combined form, with graphite below 0.2%, and to secure this result the total carbon is kept below one-fourth of the titanium content. As an illustration of the effectiveness of this relation, the following analyses are given as a result of my tests in the following table:

| Ferro-carbon titanium | Total titanium | One-fourth titanium | Total carbon | Graphitic residue |
|-----------------------|----------------|---------------------|--------------|-------------------|
| A. High-carbon.....   | Percent        | Percent             | Percent      | Percent           |
| B. Medium-carbon..    | 17.34          | 4.36                | 7.91         | 3.75              |
| C. Low-carbon.....    | 20.28          | 5.07                | 5.25         | 0.45              |
| D. Low-carbon.....    | 20.52          | 5.13                | 4.92         | 0.07              |
| E. Low-carbon.....    | 24.42          | 6.105               | 4.40         | 0.04              |
|                       | 21.78          | 5.445               | 3.78         | 0.08              |

The graphic residue as stated in the above table was determined by dissolving an analytical sample of the alloy in nitric acid, filtering off the insoluble residue which includes all graphite, and then determining the amount of carbon in that residue by combustion in the standard manner.

Since the titanium content of my improved low-carbon-ferro-carbon-titanium alloy is over four times the carbon content, or more than sufficient to form titanium-carbide with all the carbon present in the alloy, it is obvious that it differs from the previous high-carbon ferro-carbon-titanium not only in containing practically no graphite, but also in advantageously having an appreciable amount of titanium not combined with carbon but occurring as a solid solution or compound with iron or other impurities. Therefore the titanium in my new alloy exists on the whole in a more free and effective form for acting on the steel in which the alloy

is used, than in the old high-carbon alloy in which, on account of the excess of free carbon, all the titanium must necessarily be combined as carbide due to the recognized strong affinity of titanium for carbon.

5 The alloy with less than 5% total carbon and less than 0.2% graphite has been found not to increase appreciably the carbon content of steel to which it is added as a deoxidizer, whereas an 10 alloy containing free carbon or graphite has been found to carburize in an undesirable way the steel in which it is incorporated.

Hence by the use of this improved low-carbon ferro-carbon-titanium, steel manufacturers are 15 now enabled to take advantage of the purifying and other beneficial effects of titanium in soft steel containing less than 0.07% carbon without the danger of raising the carbon too high as is likely to occur when using the regular ferro- 20 carbon-titanium of 6 to 9% carbon content.

Until the development of my improved alloy, producers of soft steel containing less than about 0.07% carbon were unable to obtain the 25 advantages of titanium treatment of their steel in order to produce better rolling quality and greater cleanliness, because they found that the regular ferro-carbon-titanium containing 6 to 9% carbon, a large proportion of which is in the free or graphitic state, gave too high a carbon 30 content in the finished steel. As I have hereinbefore stated, the previously known low-carbon ferrotitaniums were too high in silicon or aluminum to be practical for use in this kind of steel.

However, with my new ferro-carbon-titanium 35 alloy containing less than 0.2% free carbon, low in silicon and aluminum, and having a close dense structure, the titanium treatment of very low-carbon steel may be accomplished successfully, with resulting benefits to the cleanliness, 40 rolling quality, and surface of the steel, and without the absorption by the steel of appreciably more carbon than it would have without any final addition of a deoxidizing or scavenging alloy.

45 The dense structure and lack of porosity of my new alloy have been found not to interfere with its solubility in molten steel, provided the titanium content is not over 25% and the carbon content is not below 1.5% or over 5%, and these 50 characteristics constitute an industrial advantage in that they tend to cause the readily crushable particles of alloy to sink into the steel bath to which they are added, instead of remaining on the surface as porous particles of the older 55 high-carbon alloy tend to float, so that my new alloy is more effectively incorporated in the steel and is not so readily lost by burning in the air at the surface of the bath.

60 I claim as my invention:—

1. An alloy capable of being cast from an electric furnace and soluble in molten steel, said alloy containing 15 to 25% titanium, 1.5 to 5% carbon and less than one-fourth the titanium content, not over 0.2% graphite, not over 3.5%

silicon and not over 3% aluminum, with the balance substantially iron.

2. An alloy capable of being cast from an electric furnace and soluble in molten steel, said alloy containing 15 to 25% titanium, 1.5 to 5% carbon substantially all in the combined form, not over 3.5% silicon, and not over 3% aluminum, with the balance substantially iron. 5

3. An alloy capable of being cast from an electric furnace and soluble in molten steel, said 10 alloy containing 1.5 to 5% carbon substantially all in the combined form, 15 to 25% titanium and always in excess of four times the carbon content and partly free from combination with carbon, not over 3.5% silicon, and not over 3% aluminum, with the balance substantially iron. 15

4. An alloy capable of being cast from an electric furnace and soluble in molten steel, said alloy containing 18 to 22% titanium, 3 to 4.5% carbon, with the titanium content partly free from combination with the carbon, 1 to 3% silicon, and 0.5 to 1.5% aluminum with the balance substantially iron. 20

5. In the manufacture of ferro-carbon-titanium alloys containing from 15 to 25% titanium 25 and less than 5% carbon by carbon reduction in a carbon-lined electric furnace, the step which consists in forming an inner lining of a refractory titanium compound on the carbon lining of said furnace by melting therein a charge containing titanium ore and carbon, said ore being in an amount in excess of that required to produce a completely fusible mass, whereby a lining of a refractory titanium compound is superposed on 30 said carbon furnace lining. 35

6. In the manufacture of ferro-carbon-titanium alloys containing from 15 to 25% titanium by carbon reduction in a carbon-lined electric furnace, the step which consists in melting therein a charge of ilmenite and carbon, said ilmenite 40 being in excess of the amount required for said alloy, to form from the molten mass a lining of a refractory titanium compound superposed on said carbon furnace lining.

7. In the manufacture of ferro-carbon-titanium alloys containing from 15 to 25% titanium by carbon reduction in a carbon-lined electric furnace, the step which consists in melting therein a charge of ilmenite, carbon and steel scrap, said ilmenite being in excess of the amount required for said alloy, to form from the molten mass 50 a lining of a refractory titanium compound superposed on said carbon furnace lining. 45

8. The method of treating effervescing low carbon steel with titanium without increasing its 55 carbon content which consists in incorporating in the molten steel a ferro-carbon-titanium alloy containing 15 to 25% titanium, 1.5 to 5% carbon and less than one-fourth the titanium content, and not over 0.2% graphite, not over 3.5% silicon 60 and not over 3% aluminum, said alloy being soluble in the molten steel and not appreciably increasing the carbon content of the effervescing steel so treated.

GEORGE F. COMSTOCK.